# EUROPEAN PATENT SPECIFICATION

(11) **EP 2 698 470 B1**
(45) Date of publication and mention of the grant of the patent: **04.07.2018**
(21) Application number: 11863535.8
(22) Date of filing: 09.09.2011
(51) Int. Cl.: D06M 13/144, A41D 31/00, D03D 15/00, D06M 11/00, D06M 11/05, D06M 13/152, D06M 101/34

(54) **METHOD FOR PRODUCING FIBROUS FABRIC, AND FIBROUS FABRIC**
VERFAHREN ZUR HERSTELLUNG EINES FASERSTOFFES UND FASERSTOFF
PROCÉDÉ POUR PRODUIRE UN TISSU FIBREUX, ET TISSU FIBREUX

(30) Priority: 13.04.2011 JP 2011089614
(43) Date of publication of application: 19.02.2014
(73) Proprietor: Komatsu Seiren Co., Ltd., Ishikawa 929-0124 (JP)
(72) Inventor: TAKAGI, Yasuharu, Ishikawa 929-0124 (JP); YONEZAWA, Kazuhiro, Ishikawa 929-0124 (JP); KOIZUMI, Makoto, Ishikawa 929-0124 (JP)
(74) Representative: Vigand, Philippe
(86) International application number: PCT/JP2011/005102
(87) International publication number: WO 2012/140704

(56) References cited:
- JP-A- 2 154 074
- JP-A- 5 311 574
- JP-A- 6 299 465
- JP-A- 2004 060 065
- US-A- 3 124 412
- US-A- 3 497 583
- US-A- 4 812 140
- DATABASE WPI Week 199238, Derwent Publications Ltd., London, GB; AN 1992-310960 & JP H04 214 484 A (KANEBO LTD) 05 August 1992

## Description

### [Technical Field]

The present invention relates to a method for manufacturing a fiber fabric having a hard texture.

### [Background Art]

Fiber fabrics made of nylon or polyester are required to have a silky handle. Accordingly, various attempts have been conducted for softening fiber fabrics. Methods for softening fiber fabrics include, for example, a method for reducing a diameter of each of fibers which make up the fiber fabric. The method for reducing the diameter of a fiber includes some methods, such as a method for directly drawing a thin fiber at a spinning stage, and a method for spinning a conjugate yarn made of nylon yarns and polyester yarns, followed by dissolving and removing polyester components using alkali agent. In addition to the above, another method can be raised in which a swelling agent, such as benzyl alcohol, for swelling nylon yarns is used to swell the nylon yarns, so that the conjugate yarn is split (Patent Literature (PTL) 1). With the aforementioned methods, thin fibers are manufactured and soft fiber fabrics can be obtained.

However, consumers' preferences have changed in recent years, and fiber fabrics having a relatively hard handle have been desirable. To cope with the above, thick yarns are used for manufacturing fabrics, or fabrics in high density are manufactured, in addition, other countermeasures are also taken.

### [Citation List]

### [Patent Literature]

[PTL 1] Japanese Unexamined Patent Application Publication No. 7-305284

JP-A-H06-299465 discloses a method for obtaining a base cloth for air bags which has high flexibility and compact foldability, said method comprising dipping a cloth of synthetic fibers such as polyamide fibers with a solution containing a swelling agent such as benzyl alcohol to swell the fibers, and then heat-treating to close the spaces between fibers.

JP-A-H04-214484 discloses a method wherein a fibrous material of nylon resin is treated with a treatment liquid comprising water and benzyl alcohol, wherein the benzyl alcohol is used in a concentration of 1 to 10 wt %, wherein thin lines of thread making up the fibers have a single yard fineness of about 0.5 to 8 denier (i.e about 0.56 to 8.89 dtex), and wherein said treatment is carried out at a temperature of 60-100°C.

### [Summary of Invention]

### [Technical Problem]

However, manufacturing thick yarns in particular causes such problems that an amount of resin used for manufacturing yarns increases, or production per one lot is not high, resulting in increase in costs for spinning yarns or manufacturing yarns. Furthermore, weaving fabrics having high density reduces productivity, which is not desirable.

Meanwhile, other measures are taken. For example, a resin for finishing fabrics hard, such as a melamine resin, is used and applied to versatile fiber fabrics. However, resins cause a fabric to have a handle unique to the resin which appears on the fabric. In addition, the resin may be pealed off from the fabric due to laundry or abrasion, so that durability of the fabric using resin is insufficient.

The present invention is made in view of the above, and aims to provide a method for manufacturing a fiber fabric. The method provides a fiber fabric having a hard handle, without using a particularly thick yarn, without manufacturing a fabric in the high density which increases loads at stages of composing and organizing the fabric, or without performing the resin treatment for hard finishing.

### [Solution to Problem]

As a result of keen examination for solving the above problems, inventors have achieved the present invention. The inventors have found that a fiber fabric having a hard handle can be obtained by performing treatment on a fabric made of nylon fibers without including polyester fibers, using a treatment liquid containing benzyl alcohol which has customarily been used, for manufacturing a soft fabric, on conjugate fibers made of nylon fibers and polyester fibers.

In other words, for solving the above problems, a method for manufacturing a fiber fabric includes performing treatment on a fabric made only of nylon fibers with a treatment liquid containing water and 30 grams to 300 grams of benzyl alcohol per liter of the treatment liquid, wherein said nylon fibers have a line of thread having a fineness ranging from 10 dtex to 500 dtex, and wherein said treatment with the treatment liquid is performed at a temperature over 100 degrees Celsius and not higher than 150 degrees Celsius.

In the method for manufacturing a fiber fabric according to the present invention, it is preferable that the treatment with the treatment liquid is performed so that the fiber fabric has a bending resistance of 100 mm or higher in at least one of a warp direction and a weft direction as measured according to a 45-degree cantilever method specified in JIS L 1096.

In the method for manufacturing a fiber fabric according to the present invention, if the fabric made only of the nylon fibers is in rope form, it is preferable that the treatment with the treatment liquid is performed at a temperature over 100 degrees Celsius and not higher than 130 degrees Celsius.

In the method for manufacturing a fiber fabric according to the present invention, if the fabric made only of the nylon fibers is in open width form, it is preferable that the treatment with the treatment liquid is performed at a temperature over 100 degrees Celsius and not higher than 130 degrees Celsius.

Preferably, the method for manufacturing a fiber fabric according to the present invention further comprises performing soaping on the fabric after the treatment with the treatment liquid, wherein said soaping is performed with hot water at a temperature from 40°C to 100°C.

A fiber fabric according to the present invention can be obtained by performing treatment on a fabric made only of nylon fibers having a line of thread having a fineness ranging from 10 dtex to 500 dtex with a treatment liquid containing benzyl alcohol, wherein the fiber fabric resulting from the treatment with the treatment liquid has a bending resistance of 100 mm or higher in at least one of a warp direction and a weft direction as measured according to a 45-degree cantilever method specified in JIS L 1096.

The fiber fabric according to the present invention can be used as a garment. Alternatively, the fiber fabric according to the present invention can be used as a storage tool.

### [Advantageous Effects of Invention]

With the method for manufacturing a fiber fabric according to the present invention, a fiber fabric having a hard handle can be obtained. The fabric resulting from the method can maintain a shape thereof without using an interlining or the like, to thereby enable a fiber product to be obtained which is excellent in design and suitable for needs.

Furthermore, in the method for manufacturing a fiber fabric according to the present invention, yarns having versatile diameters can be used. The use of such yarns provides a fiber fabric having a hard handle without specifically weaving or organizing a woven fabric or a knitted fabric in a high density. Accordingly, production costs which occur at stages of producing yarns or woven knitted products can be reduced.

### [Description of Embodiments]

Hereinafter, a method for manufacturing a fiber fabric according to the present invention is described based on embodiments.

According to the present disclosure, treatment is performed on a fiber fabric mainly made of nylon fibers using a treatment liquid containing benzyl alcohol, but according to the present invention, treatment is performed on a fiber fabric made only of nylon fibers to thereby obtain a fiber fabric having a hard handle.

Well-known nylon fibers may be used for the nylon fibers in the present invention. For example, nylon 6, nylon 10, nylon 11, nylon 12, nylon 6.6, nylon 6.10, or copolyamide made of these nylons may be used. Among them, the nylon 6 and the nylon 6.6 are preferable in terms of fiber properties, such as dyeability and strength, and a cost performance.

The fineness of each of the nylon fibers is not specifically limited, but ranges from 0.0001 dtex to 500 dtex referred to as a nano-fiber in terms of fineness of a single fiber. Furthermore, the nylon fibers may be a monofilament, a multifilament, or a staple.

The fineness of a yarn (a line of thread) may range from 0.0001 dtex to 1000 dtex but according to the present invention, the fineness of a line of thread ranges from 10 dtex to 500 dtex.

In view of cost reduction, versatility, and excellent processability, the nylon fibers are preferable which have a single fiber with the fineness of 0.1 to 10 dtex and a line of thread with the fineness of 10 dtex to 500 dtex.

Furthermore, the nylon fibers may be flat yarns or textured yarns including false-twisting, twisting, Taslan-processed yarns, or other processed yarns.

A fiber fabric made of nylon fibers according to the present disclosure is mainly made of nylon fibers. In other words, for the fiber fabric mainly made of nylon fibers, other fibers may be concurrently used, such as polyester fibers for obtaining a fiber fabric having a hard handle. However, the fiber fabric of the present invention is made only of the nylon fibers without including other fibers, such as polyester fibers, which is preferable in light of obtaining the fiber fabric having a hard handle.

It should be noted that a fiber fabric having a hard handle cannot be obtained by performing treatment on a fabric made of 50 percent polyester fibers and 50 percent nylon fibers with a treatment liquid containing benzyl alcohol. This is because that shrinkage of the nylon fibers and that of the polyester fibers largely differs upon the treatment with the treatment liquid containing the benzyl alcohol. In other words, if a fiber fabric made in combination of nylon fibers and other fibers which substantially differ from the nylon fibers in the shrinkage and are used in a large part of the fiber fabric is used, the fiber fabric with the hard handle cannot be obtained at a low cost, which should be the effect of the present invention.

Even if fibers, lines of thread, or woven knitted organizations, which are used in versatile styles, are used, the fiber fabric made only of the nylon fibers according to the present invention can have the hard handle.

Next, the method for manufacturing a fiber fabric according to the present invention is described in more detail.

In the present invention, treatment is performed on the fiber fabric made only of the nylon fibers with the treatment liquid containing the benzyl alcohol. According to the present disclosure, the treatment may be performed using a treatment liquid containing water and 10 grams to 300 grams of the benzyl alcohol per liter of the treatment liquid.

If an amount of the benzyl alcohol is less than 10 grams per liter of the treatment liquid, the fiber fabric having sufficiently hard handle may not be obtained. In accordance with the present invention, for making the handle of the fiber fabric be hardened, the amount of the benzyl alcohol is more than or equal to 30 grams per liter of the treatment liquid. On the other hand, if the amount of the benzyl alcohol exceeds 300 grams per liter, the fiber fabric is not hardened so much amount as an increased amount of the benzyl alcohol. Strength of the nylon fibers, on the contrary, may decrease. In addition, if the amount of the benzyl alcohol increases, a duty on effluent processing of the treatment liquid and the like increases.

It should be noted that benzyl alcohol which is emulsified using an emulsifying agent is preferable in view of treatment stability. To the treatment liquid containing the benzyl alcohol, a defoaming agent, a softener for treatment in bath, a friction mark prevention agent, or the like may be added.

The treatment using the treatment liquid containing the benzyl alcohol in accordance with the present disclosure can be performed at a treatment temperature of 60 to 150 degrees Celsius but according to the present invention, the treatment using the treatment liquid containing the benzyl alcohol is performed at a treatment temperature over 100 degrees Celsius and not higher than 100 degrees Celsius.

When a relatively plane fiber fabric is required, it is preferable that the treatment using the treatment liquid containing the benzyl alcohol is performed under a condition that a fiber fabric is in an open width state. For the occasion, the treatment temperature accordance with the present disclosure preferably ranges from 80 to 130 degrees Celsius.

In this case, if the treatment temperature is lower than 80 degrees Celsius, the fiber fabric with a sufficiently hard handle may not be obtained. On the other hand, depending on types of nylons, if the treatment temperature exceeds 130 degrees Celsius, strength of the fiber fabric, such as tear strength or the like, may decrease. In accordance with the present invention, for obtaining the hard handle, the treatment is preferably performed at a temperature over 100 degrees Celsius and not higher than 130 degrees Celsium, more preferably over 100 to 125 degrees Celsius, and still more preferably, over 100 to 120 degrees Celsius.

Depending on the treatment temperature or concentration of the benzyl alcohol, treatment time is preferably at a level from 5 to 180 minutes. If the treatment time is less than 5 minutes, non-uniformity may be caused in a hardened portion, or the fiber fabric having the sufficient hard handle cannot be obtained. In contrary, the treatment time over 180 minutes is not preferable for the productivity.

Furthermore, the treatment time is preferably from 7 to 120 minutes inclusive, in terms of uniformity of the hard handle, hardness of the fabric, and the productivity.

As a processing machine used for obtaining a plane fiber fabric, an atmospheric pressure jigger, a high pressure jigger can be raised.

When a fiber fabric having a bulky texture, a wrinkled texture, or a relatively intensive concave-convex surface is required, it is preferable that the treatment using the treatment liquid containing the benzyl alcohol is performed under a condition that the fiber fabric is in a rope form state. For the occasion, the treatment temperature in accordance with the present disclosure ranges preferably from 80 to 130 degrees Celsius.

In this case, if the treatment temperature is lower than 80 degrees Celsius, the fiber fabric with the sufficiently hard handle may not be obtained. On the other hand, depending on a type of nylons, if the treatment temperature exceeds 130 degrees Celsius, the strength of the fiber fabric, such as the tear strength or the like, may decrease. In accordance with the present invention, for obtaining the hard handle, the treatment is preferably performed at a temperature over 100 degrees Celsius and not higher than 130 degrees Celsius, more preferably over 100 to 125 degrees Celsius, and still more preferably, over 100 to 125 degrees Celsius.

The processing machines used for obtaining the fiber fabric having a wrinkled texture or a relatively intensive convex-concave surface include a high-pressure jet dyeing machine or a high-pressure type wince dyeing machine. It is preferable to use the jet dyeing machine for the uniformity in hardness.

The method for manufacturing a fiber fabric according to the present invention can be applied to a fiber fabric shaped in a garment, a storage tool, or the like.

For example, according to the present disclosure, when sewn products, such as garments or storage tools which are prepared using a fabric made of nylon fibers, are hardened, treatment may be performed with the treatment liquid containing the benzyl alcohol, using a washer (a drum type processing machine), at a temperature from 80 to 130 degrees Celsius for 5 to 180 minutes. It is more preferable that the treatment is performed at a temperature from 90 to 125 degrees Celsius, but in accordance with the present invention, the treatment is performed at a temperature over 100 degrees Celsius.

Heretofore, an embodiment for the method for manufacturing a fiber fabric according to the present invention is described. Here, in the present invention, it is preferable to perform soaping on the fabric made of the nylon fibers after the treatment with the treatment liquid containing the benzyl alcohol.

The soaping is washing processing with water, or hot water at a temperature of 40 to 100 degrees Celsius. Alternatively, the soaping is processing with a soaping solution prepared by adding, to water at a normal temperature or hot-water at temperature of 40 to 100 degrees Celsius, caustic soda, an alkaline agent, such as soda ash or sodium tripolyphosphate, a surfactant, or a chelating agent.

The soaping may be performed more than once. In this case, the first soaping may be performed using the soaping solution to which the alkaline agent or the surfactant is added, and the second soaping is performed using only water.

Furthermore, drying or thermal setting may be performed after the soaping, as needed. In addition to the above, dyeing finishing, water repellent finishing, antibacterial finishing, anti-odor finishing, water-absorption finishing, ultraviolet screening finishing, or antistatic finishing may be performed.

It should be noted that these processing including the dyeing finishing may be performed after sewing or other processing. Hard finishing may be supplementarily performed using polyester resin and the like.

When thermal processing, such as preliminary setting or finishing setting, is performed on the fabric made of the nylon fibers which underwent the treatment with the treatment liquid containing the benzyl alcohol, a temperature of the thermal processing may be arbitrarily set at a level of 120 to 200 degrees Celsius in view of a handle, appearance, weight, density, or other factors of the fiber fabric according to the present invention.

In the present invention, the fiber fabric having the hard handle can be manufactured with the aforementioned manufacturing method.

It is required that the fiber fabric obtained with the manufacturing method according to the present invention has bending resistance of 100 mm or higher in at least one of a weft direction and a warp direction, which is measured under a condition that an environment at the measurement is set to 20 degrees Celsius × 40 % RH, pursuant to a 45-degree cantilever method specified in "JIS L 1096". Furthermore, it is more preferable that the fiber fabric has the bending resistance of 150 mm or more in at least one of the weft direction and the warp direction. Still furthermore, it is preferable that the fiber fabric has the bending resistance of 100 mm or more both in the weft direction and the warp direction. It is more preferable that the fiber fabric has the bending resistance of 150 mm or more both in the weft direction and the warp direction.

As described above, the bending resistance of 100 mm or more provides a harder handle than a case when a traditional hard finishing is applied, which is preferable for tailoring presentation.

If the bending resistance is 100 mm or more, clothing and goods made by fabrics, which have customarily been manufactured in combination with an interlining in a separate step can be produced only using the fiber fabric according to the present invention but not using interlining. Such clothing and goods can retain shapes thereof and include a collar, a cuff, headwear, or shoes.

Furthermore, if the bending resistance is 100 mm or more, the fiber fabric according to the present invention can be used for manufacturing bags, or storage tools including a magazine rack, a storage box, a clothing case, or a pen case. In this case, the bags or the storage tools such as a storage box which retain their shapes can be obtained without coating the fiber fabric with a hard resin, or without combining, with the fiber fabric, interlinings made of cardboard boxes, plastic plates, woods, metals, or resins.

The upper limit of the bending resistance is not specifically defined. In view of a design or the like of the clothing and the bags, the fiber fabric having the necessary bending resistance may be used. According to the measurement pursuant to a 45-degree cantilever method specified in JIS L 1096, the upper limit of the bending resistance of the fiber fabric of the present invention is 150 mm. However, the fiber fabric which exceeds this upper limit can be used.

When wrinkles having the hard handle is formed in the fiber fabric, a measurement sample may be folded at the wrinkles upon measurement of the bending resistance, and the bending resistance of less than 100 mm may be measured. To cope with this, the measurement sample is taken from a portion having less effect on the measurement of the bending resistance, and the bending resistance is measured on the portion.

As described above, the fiber fabric obtained with the manufacturing method according to the present invention has the hard handle. When the fiber fabric is used to produce clothing including a jacket, headwear, and shoes, the clothing, the headwear, and the shoes having an unprecedented handle, and rough and vigorous appearance can be obtained. In addition, clothing which can retain shapes can be obtained without using the interlining.

The fiber fabric having the hard handle, which is obtained with the manufacturing method according to the present invention, is used to produce the storage tools including a bag, a pouch, a magazine rack, a storage box, a clothing case, or a pen case, to thereby obtain a new storage tool having excellent shape-retention properties in addition to a fabric handle without using the interlining.

### [Examples]

Hereinafter, a method for manufacturing a fiber fabric according to the present invention is described more specifically, based on examples and comparative examples. It should be noted that the present invention is not limited to these examples. Bending resistances in below-shown examples and comparative examples were measured in an atmosphere in which an environment at the measurement was 20 degrees Celsius × 40 % RH, pursuant to a 45-degree cantilever method specified in JIS L 1096.

### Example 1 (not forming part of the present invention)

First, Example 1 is described. In Example 1, a woven fabric (twill, 6-nylon was used for warp and weft at 100 %, in which the warp has 78 dtex / 34 filament, while the weft has 235 dtex / 34 filament. Weaving density is such that a warp density × a weft density = 244 yarns / 2.54 cm × 77 yarns / 2.54 cm) made from nylon fibers was used.

After the woven fabric was scoured, the scoured woven fabric was soaked in a treatment liquid containing 150 grams of benzyl alcohol per liter of the treatment liquid, which was prepared by injecting emulsified dispersion liquid of the benzyl alcohol into water. A temperature of the treatment liquid was raised from a room temperature to 98 degrees Celsius taking 40 minutes by using an atmospheric pressure jigger, and treatment was performed for 40 minutes with maintaining 98 degrees Celsius (open width fabric state). After that, the fiber fabric was washed with hot water at 80 degrees Celsius twice, as soaping.

Next, the fabric is dyed black with acid dye using the atmospheric pressure jigger (95 degrees Celsius for 60 minutes). Then, the soaping and fixing processing using synthetic tannin were performed on the fabric. Subsequently, drying, i.e., finishing set, is performed at 140 degrees Celsius.$The density of the obtained fiber fabric was such that the wrap density \times the weft density = 270 yarns / 2.54 cm \times 88 yarns / 2.54 cm .$

Upon measuring the bending resistance, the bending resistance in a warp direction was 148 mm while that in the weft direction was 118 mm. Thus, the fiber fabric having the hard handle was obtained.

A bag was produced using the obtained fiber fabric. The produced bag was able to maintain a three-dimensional shape only with the fiber fabric without using an interlining, and had excellent appearance.

### Comparative example 1

Next, Comparative example 1 is described. In Comparative example 1, a fiber fabric was obtained in the same manner with that in Example 1 except that the treatment with the treatment liquid containing the benzyl alcohol was not performed.$The density of the obtained fiber fabric was such that the warp density \times the weft density = 250 yarns / 2.54 cm \times 79 yarns / 2.54 cm .$

Upon measuring the bending resistance, the bending resistance in a warp direction was 42 mm while that in a weft direction was 85 mm. Thus, the fiber fabric having a soft handle was obtained.

A bag was produced using the obtained fiber fabric. The produced bag was not able to maintain a three-dimensional shape thereof without using an interlining.

### Example 2

Next, Example 2 is described. In Example 2, a woven fabric made of nylon fibers (twill, 6-nylon was used for warp and weft at 100 %, in which the warp was 355 dtex / 192 filament, while the weft was 355 dtex / 192 filament. The weaving density was such that the warp density × weft density = 95 yarns / 2.54 cm × 62 yarns / 2.54 cm) was used.

After the woven fabric was scoured, the scoured woven fabric was soaked in a treatment liquid containing 60 grams of benzyl alcohol per liter of a treatment liquid, which was prepared by injecting emulsified dispersion liquid of the benzyl alcohol into water. A temperature of the treatment liquid was raised from a room temperature to 110 degrees Celsius taking 50 minutes using a jet dyeing machine, and treatment was performed for 40 minutes with maintaining 110 degrees Celsius (rope form).

Then, the fabric was washed, as soaping, with hot water to which soda ash and surfactant were added, at a temperature of 90 degrees Celsius for 10 minutes, followed by being washed only with water and dried.

Next, preliminary setting was performed at a temperature of 160 degrees Celsius, and the fabric was dyed yellow with acid dye (105 degrees Celsius for 30 minutes). Then, fixing processing using synthetic tannin was performed on the fabric, followed by performing drying processing at 120 degrees Celsius.

Next, water repelling processing was performed using 5% solution of a fluorine-based water repelling agent including AsahiGuard AG710 (product of ASAHI GLASS CO., Ltd.), followed by performing finishing setting at 140 degrees Celsius.$The density of the obtained fiber fabric was such that the warp density \times the weft density = 116 yarns / 2.54 cm \times 85 yarns / 2.54 cm .$

Upon measuring the bending resistance, the bending density in the warp direction was 148 mm, while that of the weft direction was 117 mm. A fiber fabric having bulky feeling and a hard handle was obtained.

In addition, a coat was produced using the obtained fiber fabric. The produced coat had stiff feeling, and vigorous external appearance.

### Comparative example 2

Next, Comparative example 2 is described. In Comparative example 2, a fiber fabric was obtained in the same manner (including jet dyeing processing) with that in Example 2 except that the treatment with the treatment liquid containing the benzyl alcohol was not performed. $The density of the obtained fiber fabric was such that the warp density \times the weft density = 98 yarns / 2.54 cm \times 69 yarns / 2.54 cm .$

Upon measuring the bending resistance, the bending resistance in the warp direction is 40 mm while that in the weft direction is 35 mm. Thus, the fiber fabric having a soft handle was obtained. In addition, a coat produced with the fiber fabric had a soft handle and drape. Thus, the coat having a soft appearance was obtained.

### Example 3

Next, Example 3 is described. In Example 3, a woven fabric made of nylon fibers (a plain woven fabric, 6-nylon was used for warp and weft at 100%, in which the warp was 355 dtex / 192 filament, while the weft was 355 dtex / 192 filament. The weaving density was such that the warp density × weft density = 89 yarns / 2.54 cm × 42 yarns / 2.54 cm) was used.

After the woven fabric was scoured, the scoured woven fabric was soaked in a treatment liquid containing 50 grams of benzyl alcohol per liter of the treatment liquid, which was prepared by injecting emulsified dispersion liquid of the benzyl alcohol into water. A temperature of the treatment liquid was raised from a room temperature to 115 degrees Celsius taking 50 minutes using a jet dyeing machine, and treatment was performed for 10 minutes with maintaining 115 degrees Celsius (rope form).

Then, the fabric was washed, as soaping, with hot water to which soda ash and surfactant were added, at a temperature of 90 degrees Celsius for 10 minutes, followed by being washed only with water and dried.$The density of the obtained fiber fabric was such that the warp density \times the weft density = 109 yarns / 2.54 cm \times 59 yarns / 2.54 cm .$

Upon measuring the bending resistance, the bending density in the warp direction was 150 mm or more, while that of the weft direction was 105 mm or more. A fiber fabric having bulky feeling and a hard handle was obtained.

Next, a bag was sewn using the obtained fabric. Then, the bag was dyed red with an acid dye (at 105 degrees Celsius for 30 minutes), and underwent fixing processing using a synthetic tannin, followed by being dried at 120 degrees Celsius. The obtained bag was able to maintain a three-dimensional shape only with the fiber fabric without using an interlining, and had excellent appearance.

### Comparative example 3

Next, Comparative example 3 is described. In Comparative example 3, a fiber fabric and a bag were obtained in the same manner with that in Example 3 except that neither the treatment using the treatment liquid containing the benzyl alcohol nor dyeing processing after sewing was performed (no processing using a jet dyeing machine).$The density of the obtained fiber fabric was such that the warp density \times the weft density = 96 yarns / 2.54 cm \times 45 yarns / 2.54 cm .$

Upon measuring the bending resistance, the bending resistance in the warp direction was 56 mm while that in the weft direction was 45 mm. Thus, a fiber fabric having a soft handle was obtained.

The obtained bag was not able to maintain a three-dimensional shape thereof without using an interlining.

### Example 4

Next, Example 4 is described. In Example 4, a woven fabric made from nylon fibers (twill, 6-nylon was used for warp and weft at 100 %, in which the warp was 355 dtex / 192 filament, while the weft was 355 dtex / 192 filament. The weaving density was such that the warp density × weft density = 91 yarns / 2.54 cm × 62 yarns / 2.54 cm) was used.

After the woven fabric was scoured, the scoured woven fabric was soaked in a treatment liquid containing 40 grams of benzyl alcohol per liter of the treatment liquid, which was prepared by injecting emulsified dispersion liquid of the benzyl alcohol into water. A temperature of the treatment liquid was raised from a room temperature to 105 degrees Celsius taking 50 minutes using a jet dyeing machine, and treatment was performed for 20 minutes with maintaining 105 degrees Celsius (rope form).

Then, the fabric was washed, as soaping, with hot water to which soda ash and surfactant were added, at a temperature of 90 degrees Celsius for 10 minutes, followed by being washed only with water and dried.$The density of the obtained fiber fabric was such that the warp density \times the weft density = 120 yarns / 2.54 cm \times 85 yarns / 2.54 cm .$

Upon measuring the bending resistance, the bending density in the warp direction was 150 mm or more, while that of the weft direction was 116 mm or more. A fiber fabric having bulky feeling and a hard handle was obtained.

Next, headwear was sewn using the obtained fabric. Then, the headwear was dyed navy with an acid dye (at 105 degrees Celsius for 30 minutes), and underwent fixing processing using a synthetic tannin, followed by being dried at 120 degrees Celsius. The obtained headwear was able to maintain a three-dimensional shape only with the fiber fabric without using an interlining, and had excellent appearance.

### Comparative example 4

Next, Comparative example 4 is described. In Comparative example 4, a fiber fabric was obtained in the same manner (including processing using a jet dyeing machine) with that in Example 4 except that emulsified dispersion liquid containing the benzyl alcohol was not injected.$The density of the obtained fiber fabric was such that the warp density \times the weft density = 102 yarns / 2.54 cm \times 72 yarns / 2.54 cm .$

Upon measuring the bending resistance, the bending resistance in the warp direction was 40 mm while that in the weft direction was 30 mm. Thus, a fiber fabric having a soft handle was obtained.

The obtained fiber fabric was used to produce headwear. The obtained headwear was not able to maintain a three-dimensional shape thereof without using an interlining.

### [Industrial Applicability]

The present invention is widely usable for textile products using a fiber fabric. The textile products includes clothing, such as a coat, shoes, storage tools, such as a bag and a clothing case, or other products.

## Claims

1. A method for manufacturing a fiber fabric, comprising performing treatment on a fabric made only of nylon fibers with a treatment liquid containing water and 30 grams to 300 grams of benzyl alcohol per liter of the treatment liquid, wherein said nylon fibers have a line of thread having a fineness ranging from 10 dtex to 500 dtex, and wherein said treatment with the treatment liquid is performed at a temperature over 100 degrees Celsius and not higher than 150 degrees Celsius.

2. The method for manufacturing a fiber fabric according to Claim 1,
wherein the treatment with the treatment liquid is performed so that the fiber fabric has a bending resistance of 100 mm or higher in at least one of a warp direction and a weft direction as measured according to a 45-degree cantilever method specified in JIS L 1096.

3. The method for manufacturing a fiber fabric according to Claim 1 or 2,
wherein the fabric made only of the nylon fibers is in rope form, and
the treatment with the treatment liquid is performed at a temperature over 100 degrees Celsius and not higher than 130 degrees Celsius.

4. The method for manufacturing a fiber fabric according to Claim 1 or 2,
wherein the fabric made only of the nylon fibers is in open width form, and
the treatment with the treatment liquid is performed at a temperature over 100 degrees Celsius and not higher than 130 degrees Celsius.

5. The method for manufacturing a fiber fabric according to claim 1, said method further comprising performing soaping on the fabric after the treatment with the treatment liquid, wherein said soaping is performed with hot water at a temperature from 40°C to 100°C.

6. A fiber fabric obtained by performing treatment on a fabric made only of nylon fibers having a line of thread having a fineness ranging from 10 dtex to 500 dtex with a treatment liquid containing benzyl alcohol,
wherein the fiber fabric has a bending resistance of 100 mm or higher in at least one of a warp direction and a weft direction as measured according to a 45-degree cantilever method specified in JIS L 1096.

7. A garment including the fiber fabric according to Claim 6.

8. A storage tool including the fiber fabric according to Claim 6.

## Patentansprüche

1. Verfahren zur Herstellung eines Faserstoffes, umfassend
die Durchführung einer Behandlung auf einem nur aus Nylonfasern hergestellten Stoff mit einer Behandlungsflüssigkeit, die Wasser und 30 Gramm bis 300 Gramm Benzylalkohol pro Liter Behandlungsflüssigkeit enthält, wobei die Nylonfasern einen Fadenlauf mit einer Feinheit im Bereich von 10 dtex bis 500 dtex aufweisen, und wobei die Behandlung mit der Behandlungsflüssigkeit bei einer Temperatur von über 100 Grad Celsius und nicht über 150 Grad Celsius durchgeführt wird.

2. Verfahren zur Herstellung eines Faserstoffes nach Anspruch 1,
wobei die Behandlung mit der Behandlungsflüssigkeit so durchgeführt wird, dass der Faserstoff einen Biegewiderstand von 100 mm oder mehr in zumindest einer von einer Kettrichtung und einer Schussrichtung hat, wie nach dem in JIS L 1096 spezifizierten 45-Grad-Cantilever-Verfahren gemessen wird.

3. Verfahren zur Herstellung eines Faserstoffes nach Anspruch 1 oder 2,
wobei der nur aus den Nylonfasern hergestellte Stoff in Seilform vorliegt, und
die Behandlung mit der Behandlungsflüssigkeit bei einer Temperatur über 100 Grad Celsius und nicht über 130 Grad Celsius durchgeführt wird.

4. Verfahren zur Herstellung eines Faserstoffes nach Anspruch 1 oder 2,
wobei der nur aus den Nylonfasern hergestellte Stoff in offener Form vorliegt, und
die Behandlung mit der Behandlungsflüssigkeit bei einer Temperatur über 100 Grad Celsius und nicht über 130 Grad Celsius durchgeführt wird.

5. Verfahren zur Herstellung eines Faserstoffes nach Anspruch 1, wobei das Verfahren ferner die Durchführung einer Einseifung auf dem Gewebe nach der Behandlung mit der Behandlungsflüssigkeit umfasst, wobei die Einseifung mit heißem Wasser bei einer Temperatur von 40 °C bis 100 °C durchgeführt wird.

6. Faserstoff, der durch die Durchführung einer Behandlung auf einem nur aus Nylonfasern hergestellten Stoff mit einem Fadenlauf mit einer Feinheit im Bereich von 10 dtex bis 500 dtex mit einer Behandlungsflüssigkeit, die Benzylalkohol enthält, erzielt wird,
wobei der Faserstoff eine Biegefestigkeit von 100 mm oder mehr in zumindest einer von einer Kettrichtung und einer Schussrichtung aufweist, wie nach dem in JIS L 1096 spezifizierten 45-Grad-Cantilever-Verfahren gemessen wird.

7. Kleidungsstück, das den Faserstoff nach Anspruch 6 enthält.

8. Lagerungswerkzeug, das den Faserstoff nach Anspruch 6 enthält.

## Revendications

1. Procédé de fabrication d'un tissu fibreux, comprenant la mise en oeuvre d'un traitement sur un tissu uniquement constitué de fibres de Nylon avec un liquide de traitement contenant de l'eau et de 30 à 300 grammes d'alcool benzylique par litre de liquide de traitement, dans lequel lesdites fibres de Nylon comportent un fil linéaire ayant une finesse dans la plage de 10 à 500 dtex, et dans lequel ledit traitement avec un liquide de traitement est mis en oeuvre à une température supérieure à 100 °C et inférieure ou égale à 150 °C.

2. Procédé de fabrication d'un tissu fibreux selon la revendication 1,
dans lequel le traitement avec le liquide de traitement est mis en oeuvre de façon que le tissu fibreux ait une résistance à la flexion de 100 mm ou plus dans au moins un des sens de la chaîne et/ou de la trame, mesurée selon la méthode en porte-à-faux à 45° décrite dans JIS L 1096.

3. Procédé de fabrication d'un tissu fibreux selon la revendication 1 ou 2,
dans lequel le tissu uniquement constitué de fibres de Nylon est sous forme de corde, et
le traitement avec le liquide de traitement est mis en oeuvre à une température supérieure à 100 °C et inférieure ou égale à 130 °C.

4. Procédé de fabrication d'un tissu fibreux selon la revendication 1 ou 2,
dans lequel le tissu uniquement constitué de fibres de Nylon est de forme ouverte en largeur, et
le traitement avec le liquide de traitement est mis en oeuvre à une température supérieure à 100 °C et inférieure ou égale à 130 °C.

5. Procédé de fabrication d'un tissu fibreux selon la revendication 1, ledit procédé comprenant en outre le savonnage du tissu après le traitement avec le liquide de traitement, dans lequel ledit savonnage est effectué dans une eau chaude à une température de 40 °C à 100 °C.

6. Tissu fibreux obtenu par mise en oeuvre d'un traitement sur un tissu uniquement constitué de fibres de Nylon comportant un fil linéaire ayant une finesse dans la plage de 10 à 500 dtex avec un liquide de traitement contenant de l'alcool benzylique,
dans lequel le tissu fibreux a une résistance à la flexion de 100 mm ou plus dans au moins un des sens de la chaîne et/ou de la trame, mesurée selon la méthode en porte-à-faux à 45° décrite dans JIS L 1096.

7. Vêtement contenant le tissu fibreux selon la revendication 6.

8. Outil de stockage contenant le tissu fibreux selon la revendication 6.
